

# United States Patent

[11] 3,617,220

[72] Inventors **Donald R. Moore**  
**Rutherford;**  
**Stanley E. Ross, Passaic; Giuliana C.**  
**Tesoro, Dobbs Ferry, all of N.J.**  
[21] Appl. No. **19,488**  
[22] Filed **Mar. 13, 1970**  
Division of Ser. No. 721,145, Apr. 15,  
1968, Pat. No. 3,527,564.  
[45] Patented **Nov. 2, 1971**  
[73] Assignee **J.P. Stevens & Co., Inc.**  
**New York, N.Y.**

[54] **PROCESS FOR CARBONIZING CELLULOUSIC  
FIBROUS SUBSTRATES**  
3 Claims, No Drawings  
[52] U.S. Cl. .... **23/209.5,**  
8/116, 8/116.2  
[51] Int. Cl. .... **C01b 31/07**  
[50] Field of Search. .... **23/209.5,**  
**209.1, 209.4; 8/116, 116.2; 117/136, 138**

[56] **References Cited**  
UNITED STATES PATENTS  
3,235,323 2/1966 Peters..... 8/116.2  
3,294,489 12/1966 Millington et al..... 23/209.4  
OTHER REFERENCES  
Schmidt et al. "Chem. Eng. Progress" vol. 58, No. 10, Oct.  
1962, pages 42-43  
Primary Examiner—Edward J. Meros  
Attorneys—Michael T. Frimer and Charles Stein

**ABSTRACT:** A process for improving the thermal carbonization of cellulosic substrates comprising treating said substrates prior to carbonization with a catalytic amount of at least one compound selected from esters of phosphoric acid, esters of phosphorothioic acid, phosphoramidic acids, alkylphosphoramidic acids, alkylphosphonic acids, alkylphosphonothionic acids, and phosphonitrile amide derivatives and heating said treated substrates until a carbonized product having a carbon content of at least 50 percent weight carbon is produced.

## PROCESS FOR CARBONIZING CELLULOSIC FIBROUS SUBSTRATES

This application is a division of copending U.S. application Ser. No. 721,145, now U.S. Pat. No. 3,527,564 filed Apr. 15, 1968.

This invention concerns reagents useful as catalysts for the pyrolytic transformation of carbon-containing substrates to carbon products.

More particularly, this invention relates to novel catalysts employed during the carbonization and graphitization of cellulosic substrates to effect product and process improvement.

ulosic substrates to effect product and process improvement. Carbonization as used herein refers to thermally actuated processes which transform a carbon-containing substrate to a carbon product. These carbon products include both carbon and graphite materials whose carbon (or graphite) content ranges from about 50 percent by weight to almost 100 percent by weight.

The term cellulosic as used herein refers to substrates comprising natural cellulose or its modified derivatives. These include cotton, linen, hemp, jute, flax, wood, cuprammonium rayon, viscose and the like. These cellulosics can be employed unblended or in the form of blends with noncellulosic materials. The latter include, but are not limited to the acrylics, polyesters, and polyamides. The substrates can be used in the form of their yarns, fibers, or threads as well as in the form of materials such as woven cloths, knitted fabrics, webs, laminates, or any other fabricated form utilizing textile fabricating processes.

The carbonization of carbon-containing substrates to produce carbon or graphite filaments dates back more than 60 years. More recently, stimulated by the need in the aerospace program for strong, lightweight and inert materials, there has been a resurgence of carbonization and graphitization research. Particularly of interest are programs in which carbon-containing textile materials such as cellulosic yarn and cloth have been pyrolyzed under carefully controlled conditions to produce carbon products retaining a substantial portion of the desirable characteristics of the original textile substrate. For example, the products are lightweight, have good flexibility, and are nontoxic. Further, as compared to the original cellulosic substrate, they have improved chemical inertness and dimensional stability. Finally, in contrast to the cellulosics, they possess outstanding resistance to flammability and good high-temperature ablation.

Most of the published procedures for carbonizing cellulosics disclose lengthy stepwise heating processes to produce the final product. Initially, the substrate is slowly heated to temperatures ranging from about 200° C. to 30° C. followed by a final and brief heating step at high temperatures ranging from about 550° C. to 2,000° C. or even higher. Not only are equipment and labor costs high but the prolonged heating at elevated temperatures reduces yields and requires the use of inert atmospheres to prevent combustion of the substrate. As a result of these factors, the cost of carbonized articles is exceedingly high and the widespread use of the carbon products has been kept to a minimum.

It has been known for some time that pretreatment of the cellulosic substrate with appropriate catalytic reagents can reduce the time required for completion of the carbonization cycle. Recently, the use of certain mineral acids and acidic salts such as phosphoric acid and diammonium hydrogen phosphate as carbonization catalysts have been described in patents (U.S. Pat. Nos. 3,235,323 and 3,305,315). The patentees have indicated that the use of these catalysts during carbonization produces improved carbon products compared to products obtained without catalysts. However, even when a superior catalyst such as diammonium hydrogen phosphate  $[(\text{NH}_4)_2\text{HPO}_4]$  is used, difficulties are encountered. For example, even when the catalyst is used, a comparatively lengthy heating cycle is required to obtain a carbonized product having acceptable properties. Further, diammonium hydrogen phosphate should be applied at near boiling temperatures. A major advance in the art would be the development of new

catalytic reagents which could be applied at moderate temperatures ( $20^{\circ}$  C.- $50^{\circ}$  C.) and which would substantially reduce the heating time required for carbonization compared to diammonium hydrogen phosphate. In addition, a truly superior catalyst would lend itself to simple, routine application techniques and would produce a carbon product having improved physical properties in good yield. In addition, the catalyst should be relatively simple to prepare and purify, and would function at effectively low concentrations.

It is, therefore, an object of this invention to disclose a novel and superior class of catalysts for the carbonization of cellulosic substrates.

A more particular object of this invention is the development of carbonization catalysts which substantially reduce carbonization time compared to presently utilized catalysts such as diammonium hydrogen phosphate.

Another specific object of this invention is the development of novel water-soluble carbonization catalysts which readily lend themselves to simplified application procedures conducted at moderate temperatures.

An additional specific object of this invention is the utilization of the inventive catalysts to prepare carbon products having improved properties.

Other objects of this invention will become apparent to those skilled in the art after a reading of this application.

The above objects are realized by the treatment of a cellulosic substrate prior to complete carbonization with a class of organic materials that will decompose during

carbonization catalysts to be described more fully below.

In practice, a cellulosic substrate is treated with one or more catalysts selected from the groups consisting of:

catalysts selected from the groups consisting of:



wherein G is selected from the group consisting of —OR or



R is an alkyl radical having from one to four carbon atoms, R' and R<sup>2</sup> which can be the same or different at any given time are selected from hydrogen and R; L is selected from the group consisting of alkyl radicals containing from one to four carbon atoms, halogenated alkyl radicals containing from one to four carbon atoms, and G; and Z is selected from the group consisting of oxygen and sulfur; in an amount sufficient to incorporate at least a catalytic quantity\* of catalyst into the substrate to be carbonized.

\* While a catalytic quantity of catalyst is a variable depending upon the catalyst and reaction conditions employed, in general this quantity varies between 2 and 30% by weight of catalyst(s), based on the weight of the substrate.

While the above two classes of compounds provide satisfactory catalysts for the carbonization of carbon-containing substrates, in any large group for various reasons some members of the group are preferred to others. In the instant case the

The group are preferred to others. In the instant case the preferred catalyst are selected from the group consisting of phosphoric triamide, phosphorothioic triamide, phosphonitrile amide cyclic trimer, diethyl methylphosphoramidate, and diethyl ethylphosphoramidate. These compounds are the preferred catalysts for carbonizing carbon-containing substrates because they reduce the carbonization time required in the first heating stage and produce

carbon products having outstanding properties in most instances in high yield.

A secondary favored group of compounds which, while excellent catalysts, are not as outstanding as the preferred catalysts, are those compounds selected from the group consisting of methylphosphonic diamide and (chloromethyl)phosphonothionic diamide. These catalysts generally give good yields of carbonized products and the products have superior properties. The trialkyl phosphates as exemplified by triethyl and trimethyl phosphate, N,N',N"-trimethylphosphoric triamide, and diethyl isopropylphosphoramidate, form a tertiary group of very good catalysts which give lesser yields of a product having somewhat less desirable properties.

The residuum of the compounds included within the two broad classes of catalysts are least preferred for a variety of reasons including poor water solubility, poorer properties, and the requirement for longer residence times.

After treatment with catalyst, the treated substrate is then heated to effect removal of the volatiles to obtain a permanently dehydrated material having a carbon content of at least 50 percent by weight carbon. This black appearing, devolatilized and heat-treated material can be utilized as an electrical insulator or can be further heated to produce a carbonized or graphitized material having a carbon content of at least 85 percent and up to 100 percent by weight carbon. The latter products are useful as electrically conductive materials and when utilized in resin-bonded laminates are exceedingly valuable in fabricating ablative composites.

In the preferred practice, a fibrous cellulosic textile substrate such as cotton or rayon cloth or yarn is treated with an aqueous solution (1-10 percent active solids) of at least one catalyst selected from the above-described, preferred group until a pickup of 150-300 percent based on the dry weight is obtained. The treated cellulosic substrate is dried to a moisture content of approximately 8-12 percent and heated at 200°-300° C. until a black fibrous substrate having a carbon content between 50-65 percent by weight carbon is produced. Ordinarily, depending upon the heating temperature, and the efficacy of the catalyst, the initial carbonization takes between 3 and 12 minutes. Substrates treated with diammonium hydrogen phosphate require between 8-12 minutes when carbonized at this temperature range.

As noted earlier, the product containing 50-60 percent by weight of carbon can be further carbonized to produce a product containing 85 percent by weight or higher carbon content. This is most easily accomplished by heating the carbonized substrate briefly above about 1,000° C. in a nonoxidizing atmosphere. The upper temperature range is primarily limited by whether a carbon or graphite product is desired. The precise residence time required for the final carbonization is a variable depending primarily on the second carbonization temperature and to some extent on the catalyst employed during carbonization. When phosphoric triamide (one of the preferred catalysts of this invention) is employed as catalyst, good results have been obtained by heating the black uniformly lustrous fibrous substrate for from 20 to 120 seconds at the 1,300° C.-1,500° C. range. After the final carbonization (or graphitization) is complete the fibrous carbon product is cooled, collected and scoured or otherwise finished depending upon the intended end use.

As described supra, the preferred carbon-containing substrates are cellulosics, particularly those broadly described as regenerated cellulose or rayon. The fibrous rayon can be in the form of a cloth (woven, knitted or felted), nonwoven random layed fibrous or needlepunched batts, felts, fabrics or tissues formed of staple, fibers, yarns, rovings, continuous filament tows and the like.

The cellulosic substrate can be in the form of yarns, fibers or filaments (or the textile fabrics made from these) whose diameter can vary widely. An especially suitable range lies between about 5 to about 30 microns in diameter.

As the preferred catalysts of this invention are water soluble, it is most convenient to utilize the one or more catalyst employed in the form of their aqueous solutions. Water solubility is an important attribute of a preferred catalyst since it permits the use of simple application techniques and existing apparatus. However, if desired, emulsions or suspensions of the soluble or less soluble catalyst(s) in nonaqueous solvents or mixtures of nonaqueous solvents with water can be employed. Textile adjuvants such as surfactants, emulsifiers, stabilizers, or the like can be present in the treating solution if desired.

The mode of applying the treating solution is not critical to the success of this invention. Any application technique utilized in the textile art can be employed. These include, but are not limited to, padding, brushing, spraying, coating, and the like. As the catalysts can be applied at moderate temperatures, a convenient mode of applying them to yarn is to run the yarn continuously through an aqueous bath containing catalyst and removing excess solution to achieve the desired wet pickup. When cloth is used as the substrate, comparable application methods may be employed.

After the application is complete the treated substrate is dried. The drying step can be air dried or heat assisted. It can be conducted as a separate step or can be incorporated as part of the heating cycle.

Similarly the carbonization or graphitization can be conducted in two or more stages or as a continuous stage. No special heating source is needed. Conventional muffle or tube furnaces can be used modified or as marketed.

In the initial carbonization phase (up to about 50-60 percent by weight carbon content) the use of the inventive catalysts precludes the need for heating in a nonoxidizing atmosphere to prevent combustion. However, the subsequent high temperature heating step where the carbon content runs from 85 percent by weight and higher requires a nonoxidizing atmosphere (less than 10 percent by weight oxygen). This can be accomplished by heating the substrate in a nitrogen, carbon dioxide, or noble gas atmosphere (or mixtures thereof) or by diluting air with diluents such as steam, ammonia, or the above enumerated inert gases until the desired environment is obtained.

The final carbonized or graphitized carbon product can be washed or scoured to remove undesirable contaminants or salts if desired. In the former case the product can be batchwise or continuously immersed in water while in the latter instance soaps or detergents can be added to the bath if convenient.

Having described the inventive process generally, it only remains to disclose specific embodiments of the use of the catalysts of this invention in carbonization and graphitization procedures. A description of the evaluation techniques precedes the specific embodiments.

#### 5 I. Criteria Used to Evaluate the Carbonization Catalysts of this Invention

In order to evaluate the carbonization catalysts objectively and to compare them in efficacy to the Prior Art Standard (diammonium hydrogen phosphate), the following criteria were used:

- 65 A. Length of time required to carbonize satisfactorily to a carbon product when the first stage of carbonization is carried out at a relatively low temperature, i.e., about 260° C.
  - B. Tensile strength of the substantially carbonized (85 percent carbon or over) yarn.
  - C. Modulus of elasticity of the substantially carbonized yarn.
  - D. Percent by weight carbon content of the substantially carbonized product.
  - E. Electrical resistivity of the substantially carbonized yarn.
- In all instances, diammonium hydrogen phosphate was used as the control.
- 70 75 A. Specific Two-Stage Carbonization Process Used





J. Diethyl ethylphosphoramidate,  
 $\text{OP}(-\text{OC}_2\text{H}_5)_2$   
 $\text{HN C}_2\text{H}_5$

(applied as a 5% solution).

| Residence times at lower temperatures, min. | Carbonization temperature |                   |       |
|---------------------------------------------|---------------------------|-------------------|-------|
|                                             | 254° C.-1,372° C.         | 260° C.-1,372° C. | 3.5   |
| 7                                           | 5.25                      | 3.5               |       |
| 10                                          |                           |                   |       |
| Denier                                      | 900                       | 816               | 1,012 |
| Breaking strength, grams                    | 2,490                     | 2,452             | 2,178 |
| Tensile strength, g./d.                     | 2.77                      | 3.00              | 2.15  |
| Elongation, percent                         | 1.69                      | 1.83              | 1.61  |
| Modulus of elasticity, g./d.                | 211                       | 202               | 169   |
| Carbon content, percent                     | 99.6                      | 98.7              | 95.2  |

K. Diethyl isopropylphosphoramidate,  
 $\text{OP}(-\text{OC}_2\text{H}_5)_2$   
 $\text{HNCH}(\text{CH}_3)_2$

(applied as a 5% solution).

| Carbonization temperature, ° C.           | 260-1,372 |
|-------------------------------------------|-----------|
| Residence time at lower temperature, min. | 5.25      |
| Product properties:                       |           |
| Denier                                    | 830       |
| Breaking strength, grams                  | 1,302     |
| Tensile strength, g./d.                   | 1.59      |
| Elongation, percent                       | 0.77      |
| Modulus of elasticity, g./d.              | 245       |
| Carbon content, percent                   | 93.0      |

L. Methylphosphonic diamide,  
 $\text{OP}(\text{NH}_2)_2$   
 $\text{CH}_3$

(applied as 3½% solution).

| Residence times at lower temperatures, min. | Carbonization temperatures |                   |
|---------------------------------------------|----------------------------|-------------------|
|                                             | 271° C.-1,372° C.          | 277° C.-1,372° C. |
| 7                                           | 5.25                       |                   |
| 10                                          |                            |                   |
| Denier                                      | 1,014                      | 1,002             |
| Breaking strength, grams                    | 2,270                      | 2,014             |
| Tensile strength, g./d.                     | 2.15                       | 2.01              |
| Elongation, percent                         | 1.34                       | 1.23              |
| Modulus of elasticity, g./d.                | 204.7                      | 210.8             |
| Carbon content, percent                     | 93.0                       | 93.5              |

The results using fabric substrates are as follows:

M. A woven fabric consisting of 1650/720/2Z rayon yarns in a 21×22 (warp×filling) construction was impregnated with a 3.5 percent by weight aqueous solution of N,N',N'''-trimethylphosphoric triamide. After drying, the fabric was exposed to temperatures in the range of 288° C.-316° C. for a period of nine minutes. At this stage of carbonization the fabric had a carbon content of 60.8 percent. Other combinations of time and temperature produced the same result. The fabric was then passed through a zone heated to 1,200° C. for a period of approximately 20 seconds. During this time the carbon level increased to 88 percent. The carbonized fabric was flexible and exhibited a high tensile strength in both warp and filling directions.

N. The same fabric was impregnated with a 5 percent by weight solution of phosphoric triamide and exposed to a heating cycle consisting of a gradual increasing temperature from 230° C. over a period of fifteen minutes. The fabric was then exposed to a temperature of 1,538° C. for a period of 20 seconds. The resultant carbonized fabric had a carbon content of 95 percent. The fabric had excellent tensile strength and was flexible and uniformly lustrous.

O. Comparable results were obtained on the same fabric treated with 5 percent by weight aqueous solutions of the

following catalysts: phosphorothionic triamide, (chloromethyl)phosphonothionic diamide, phosphonitrile amide cyclic trimer, trimethyl phosphate, triethyl phosphate, diethyl methylphosphoramidate, diethyl ethylphosphoramidate, diethyl isopropylphosphoramidate, and methylphosphonic diamide.

Since the disclosure in U.S. Pat. No. 3,294,489 (Millington) states that flameproofing agents generally, particularly phosphates, borates, and chlorides would be effective catalysts, several known flameproofing agents were evaluated and were not found to be effective catalysts. For example, a boric acid-metaborate mixture, even at the 5 percent concentration level did not give a satisfactory product at carbonization temperatures of 260° C., 275° C., 288° C., at 10 minutes' residence time followed by the usual 20 seconds at 1,372° C. Similarly, a borax-boric acid mixture at 5 and 10 percent concentration at 288° C. for periods of 6 and 9 minutes followed by exposure at the usual 1,372° C. for 20 seconds did not give a product of over 82 percent carbon and the product was too brittle for testing. The above data confirmed that the choice of catalyst even from the class of flame retardants is an empirical selection and successful catalysts cannot be predicted in advance.

As the above data indicate, the novel catalysts of this invention are advantageous in several respects. In some instances they offer advantages over prior art catalysts exemplified by diammmonium hydrogen phosphate. For example, all of the catalysts can be applied at room temperature and most of the catalysts function well even at much shorter residence times in the initial carbonization. The lower temperature application is more convenient and reduces safety hazards while the lower residence times effect substantial savings in labor and product costs. The preferred compositions such as phosphoric triamide, phosphorothioic triamide, phosphonitrile amide cyclic trimer, diethyl ethylphosphoramidate, and diethyl methylphosphoramidates not only reduce residence time considerably but actually yield a product having superior physical properties.

As the various examples and discussion in the specification have previously indicated, numerous changes and modification of reagents and reaction conditions can be made without departing from the inventive concept. The metes and bounds of the invention are best described by the claims which follow

What is claimed is:

1. A process for improving the thermal carbonization of cellulosic fibrous substrates comprising treating said substrates prior to carbonization with at least a catalytic amount of a catalyst of the formula



wherein

R' and R<sup>2</sup> are selected from the group consisting of hydrogen and alkyl of 1 to 4 carbon atoms and heating said treated substrates until a carbonized product having a carbon content of at least 50 percent by weight carbon is produced.

2. The process of claim 1 wherein the treated substrate is heated until a carbonized product having a carbon content of at least 80 percent by weight carbon is produced.

3. The process of claim 1 wherein the catalyst is phosphonitrile amide cyclic trimer.

\* \* \* \* \*

UNITED STATES PATENT OFFICE  
CERTIFICATE OF CORRECTION

Patent No. 3,617,220 Dated November 2, 1971

Inventor(s) Giuliana C. Tesoro, Donald R. Moore and Stanley E. Ross

It is certified that error appears in the above-identified patent and that said Letters Patent are hereby corrected as shown below:

In the Abstract, next to last line after "50 percent" insert -- by --; Col. 1, line 50, "200°C. to 30°C." should read -- 200°C. to 300°C.--; Col. 6, line 4, "(1969)" should read -- (1960) --; Col. 6, line 5, "cacording" should read -- according -- ; Col. 6, lines 13 and 15, "hezaamino" should read -- hexaamino --; line 15 at the end of the line "heza--" should read -- hexa --; Col. 6, line 31 "75=25" should read -- 75:25 -- ; Col. 9, line 26, "1302" should read -- 1320 --; Col. 9, line 53, "316<vc." should read -- 316°C. --; Col. 10, line 1, "phosphorothionic" should read -- phosphorothioic --.

Signed and sealed this 19th day of March 1974.

(SEAL)

Attest:

EDWARD M. FLETCHER, JR.  
Attesting Officer

C. MARSHALL DANN  
Commissioner of Patents